

April 14, 1970

KATSUO MAKINO ET AL

3,506,595

PHOTOCONDUCTIVE INSULATING MATERIAL

Filed Oct. 31, 1966



FIG.1



FIG.2

INVENTORS  
KATSUO MAKINO  
IWAO SAWATO

BY

*Sughrue, Rothwell, Mion, Zinn & Macpeak*  
ATTORNEYS

1

3,506,595

PHOTOCONDUCTIVE INSULATING MATERIAL  
Katsuo Makino and Iwao Sawato, Odawara-shi, Japan,  
assignors to Fuji Shashin Film Kabushiki Kaisha,  
Kanagawa, Japan

Filed Oct. 31, 1966, Ser. No. 590,800

Claims priority, application Japan, Oct. 30, 1965,  
40/66,529

Int. Cl. G03g 5/00, 5/08

U.S. Cl. 252—501

3 Claims

## ABSTRACT OF THE DISCLOSURE

A photoconductive insulating material comprising cadmium sulfide and cadmium carbonate photoconductive powder having metal iodide incorporated therewith, the molar ratio of the metal iodide to the cadmium sulfide and cadmium carbonate being approximately 0.01 to 0.1. The powder is dispersed through an electrically insulating binder.

This invention relates in general to a photoconductive insulating material and more particularly to an electro-photographic photosensitive member having high photosensitivity comprising photoconductive fine powders dispersed in a binder.

The photoconductive insulating member is herein defined as a member the electrical resistance of which is higher than  $10^8$  ohm-cm. in a place where no radiation exists, but the resistance of which is decreased when it is irradiated by light or other radiations.

In electrophotography, various kinds of processes have been conducted, but brief explanations will be given hereafter on the most widely known and employed process for convenience and for a better understanding of the subject matter of this invention. An electro-photographic photosensitive member is first electrostatically charged by corona discharge in a dark place. The charged member is then exposed to a light image to be reproduced by a conventional exposing method. The charges leak off in proportion to the intensity of light to which any given area is exposed. After such exposure, a latent electrostatic image is formed on the surface of the member. Development of the latent image is carried out by contacting the member bearing the latent electrostatic image with electrostatic marking particles. These particles adhere to the areas where the electrostatic charges remain, forming a powder image corresponding to the electrostatic image. The powder image can then be fixed directly onto the surface of the photosensitive member or transferred to a sheet of transfer material and fixed thereon by a suitable method. In the case of transferring the powder image, the residual powder on the surface of the photosensitive member is cleaned off and the member is used repeatedly. The process described above is the most popular one. Though various kinds of electro-photographic processes have been employed besides the aforesaid process, the essential properties of the photoconductive insulating layer of the photosensitive member are substantially identical in such processes.

The "potential acceptance" is hereinafter defined to be the surface potential of an electro-photographic photosensitive member when the member is charged electrostatically by, for instance, corona discharge; and the "half decay exposure time" is defined to be the period of time required for the surface potential to reduce to half of the initial potential during light exposure. An electro-photographic photosensitive member of higher potential acceptance and of the shorter half decay exposure time is desirable. These properties are deteriorated in general when the photosensitive member is irradiated with intense

2

light before being charged. In particular the potential acceptance becomes lower. This is the so-called light fatigue or pre-exposure effect. A higher potential acceptance generally corresponds to a higher dark resistance of a photoconductive member, although there does not exist a clear one-to-one correspondence between them. The sensitivity of the photocurrent of a photoconductive member corresponds to the half decay exposure time thereof. We, the inventors, have found that fine particles of a cadmium sulfide-cadmium carbonate photoconductor are excellent electro-photographic photosensitive material. The photoconductive insulating member having the above-mentioned powders can be charged in positive or negative, by a suitable corona discharging and the like, and shows substantially the same potential acceptance as well as substantially the same photosensitivity (exactly speaking, a little higher sensitivity in the negative polarity than that in the positive polarity) to both polarities. These powders are, however, inferior to vitreous selenium in photosensitivity and light fatigue, as described hereinafter, and are insufficiently used in place of the vitreous selenium, and hence is required that their properties be improved.

Hereupon, in an automatic copying machine a higher photosensitivity is imposed upon an electro-photographic photosensitive member. Further, electro-photographic members to be used in copying machines where a transfer process is used are required to have sufficient electro-photographic properties and mechanical strength to endure repeated use. The inventors have studied electro-photographic photosensitive members mainly consisting of a photoconductive powder of cadmium sulfide, and of a cadmium sulfide-cadmium carbonate photoconductive powder dispersed in a binder as an electro-photographic photosensitive member to be used repeatedly in an automatic copying machine, but their properties are found to be inferior to a photosensitive member mainly consisting of vitreous selenium. The study has further been carried out in order to improve their properties and the incorporation of iodine has been found to be effective to satisfy the requirements. Namely, by adding iodine, a photosensitive member comparable to the vitreous selenium photosensitive member for the repeated use in an automatic copying machine has been obtained. However, in the case of adding elementary iodine there are some difficulties in the production of members having stable properties and constant composition, since some amount of iodine will be lost during the addition or drying processes owing to its high vapour pressure.

In order to overcome the above difficulty in the manufacturing process, the inventors have studied a method where iodine is added as a form of a metal iodide and have obtained satisfactory results. Therefore, this invention relates to the photoconductive insulating material which is produced by dispersing in an electrically insulating binder the photoconductive powders mainly comprising a cadmium sulfide-cadmium carbonate photoconductor having a form of, for example,



60 together with a metal iodide.

The metal iodides used in the invention may be water soluble and/or organic solvent soluble ones. For examples, there are lithium iodide, magnesium iodide, beryllium iodide, bismuth iodide, tungsten iodide, cesium iodide, strontium iodide, tin iodide, potassium iodide, cadmium iodide, antimony iodide, aluminum iodide, and zinc iodide. These compounds may be incorporated in the cadmium sulfide-cadmium carbonate photoconductive powder as a solution thereof, i.e., the powder may be impregnated with the metal-iodide solution and dried. In another way, the photoconductive powder may be treated

with the metal iodide vapour to adsorb it or diffuse it into the powder particles. A metal iodide which cannot be dissolved into water or organic solvents, such as lead iodide, may be also employed in this invention and, in such a case, the iodide may be incorporated in the photoconductive powder by heating the powder in the vapour of the iodide formed by heating it.

The cadmium sulfide-cadmium carbonate photoconductive powder used in the present invention may be prepared by mixing an aqueous solution containing a carbonate ion and a sulfur ion with an aqueous solution containing a cadmium ion, or by mixing an aqueous solution containing a carbonate ion with an aqueous solution containing a cadmium ion in the presence of hydrogen sulfide, and, thereafter, baking the thus precipitated reaction product. As the cadmium salt there may be used a cadmium halide, cadmium sulfate, cadmium nitrate and the like and, as the carbonate, there may be used sodium carbonate, potassium carbonate, ammonium carbonate and the like. The cadmium sulfide-cadmium carbonate photoconductive material used in this invention is not a simple mechanical mixture of cadmium sulfide particles and cadmium carbonate particles, but it is considered that one particle of the powder consists of both cadmium sulfide and cadmium carbonate although its particle structure and/or its crystal structure have not yet been understood.

In X-ray diffraction analysis of the photoconductive material the diffraction lines of cadmium sulfide and cadmium carbonate are observed independently. But their diffraction lines are broad and diffuse, which indicates the crystallinity being not so high. The ratio of both components is preferably that  $n$ , in the form of



is less than 4.

The binder used in the invention should be electrically insulative and should not be chemically, electrically and physically poisonous to the photoconductive powder. For example, a synthetic resinous binder is preferable. And as the resinous binder, there are room temperature setting types, catalytically setting types, and thermosetting types of resinous binders, and they may be used in accordance with its purpose of usage. Various combinations of the above binder materials may be also employed. Further, as the binder, a low melting glass (a kind of inorganic polymer) may also be used.

When elementary iodine is added to the photoconductive powder, it is required that special care be given to the atmospheric conditions, in drying and heat treatment processes, for preventing the iodine from being volatilized off, but such a care is not needed when using metal iodide compounds in accordance with the present invention. The photoconductive powder incorporated with the metal iodide is dispersed in a binder to form a photoconductive insulating member, whose properties are similar and comparable to the member incorporated with iodine as well as to the member of vitreous selenium. The photosensitivity of the member thus prepared becomes several times higher and the light fatigue thereof decreases in comparison to the member without any iodine and metal iodide. Though explanations are herein given mainly about a layer form photoconductive insulating member, other forms of the member may be presented. Instead of coating the dispersion of the photoconductive powder in the binder on a support, such as a metal plate or a paper sheet, the dispersion may be cured and ground into comparatively large particles, ranging from several microns to several hundred microns, which may be used, as it is, as a photoelectric photosensitive material.

Moreover, the electrophotographic photosensitive material of the invention is superior for the photosensitive member on which the powder image is directly fixed.

Further, the photoconductive insulating member of the invention can be used not only for the photosensitive

material in various kinds of electrophotographic processes, but also for the photosensitive material in various kinds of photoelectric converting processes. For instance, it may be used for the photosensitive material in a photocell, a light image convertor, such as a light image amplifier and a vidicon, a phototape or X-ray-to-visible image convertor, etc.

In this specification, explanations have been given mainly about the photoconductive insulating member which is used as the electrophotographic photosensitive member, but the applications of the invention should not be restricted within these explanations and illustrations.

The following examples are now presented as detailed illustrations.

#### Examples 1-4

In accordance with the prescriptions described in Table 1, shown below, 450 mls. of an ethyl alcohol solution of cadmium iodide was mixed with a cadmium sulfide-cadmium carbonate powder of  $\text{CdS} \cdot 1.5\text{CdCO}_3$ . That is, the powder was dispersed in pure ethyl alcohol, into which an ethyl alcohol solution of cadmium iodide was added dropwise with agitating. The slurry, thus obtained, was then well agitated and dried at a temperature of 80° C. to 90° C. for 24 hours. About half of each dried powder in Example 1 or Example 2 was further baked in a glass bottle in an air oven at a temperature of 200° C. for 24 hours to prepare the powders of Example 3 or Example 4, respectively. Thereafter, in accordance with the prescription described in Table 1, each powder thus treated was mixed and dispersed in a binder in a porcelain ball mill to make a photosensitive paint, the binder used herein being a thermosetting acrylic resinous binder named "Magicron No. 200 Clear" manufactured by Kansai Paint Co., Ltd. From the thus prepared photosensitive paint electrographic photosensitive members having various thicknesses were prepared by coating on aluminum sheets, drying them and baking them at the temperatures of 150° C., 200° C., and 250° C.

The measurements of the potential acceptance and the half-decay exposure time of the electrophotographic photosensitive members thus obtained were carried out by charging them by -7.0 kilovolts corona discharge. The potential acceptance and the half-decay exposure time were increased as the thickness of the photosensitive layer was increased. Therefore, the relation of the potential acceptance to the half-decay exposure time of each of the photosensitive members which were made of the same photosensitive paint and by the same baking condition formed one relation curve. From the curves thus obtained from the various kinds of photosensitive paints and by the various kinds of baking conditions, the half-decay exposure times which correspond to the potential acceptance of 500 volts were estimated. The half-decay exposure times thus obtained for various kinds of the photosensitive members are listed in Table 1 as S-HDET. The baking conditions A, B, and C, in Table 1 denote the baking temperatures and the baking times, i.e., at 150° C. for 30 min., at 200° C., for 60 min., and at 250° C. for 30 min., respectively. By these examples the fact that the photosensitivity increased with the cadmium iodide concentration was confirmed, the photosensitivity being considered to correspond to the reciprocal of the half-decay exposure time. In Examples 1 and 3, where the quantity of iodide added was small, the photosensitivity increased as the baking temperature became higher. On the contrary, in Examples 2 and 4, where large quantities of cadmium iodide were added, the photosensitivity decreased as the baking temperature increased. This tendency is evident in Example 4, where the powder incorporated with cadmium iodide was fired. Anyhow, the highest photosensitivity was reached at the baking condition A in Example 4, which can be thought to indicate that sufficient photosensitivity can be obtained, even if there is no baking of the coating for curing of the binder

material. In the case of charging in a positive polarity, the same tendency as with charging in a negative polarity was observed, though the photosensitivity was a little lower, as listed in Table 1.

TABLE 1  
[Relation between the preparation conditions of sample in Examples 1-4 and S-HDET]

| CdS·1.5CdCO <sub>3</sub><br>Powder (grams) | CdI <sub>2</sub> Mol<br>percent<br>added | Firing condition      | Binder<br>(Solid<br>Part)<br>(grams) | (-7.0 kv.) (sec.) |     |      | (+)7.0 kv.) (sec.) |      |     |
|--------------------------------------------|------------------------------------------|-----------------------|--------------------------------------|-------------------|-----|------|--------------------|------|-----|
|                                            |                                          |                       |                                      | A                 | B   | C    | A                  | B    | C   |
| Example 1                                  | 60                                       | 1.0                   | 30                                   | 3.1               | 2.4 | 2.0  | 3.9                | 2.45 | 2.6 |
| Example 2                                  | 60                                       | 10.0                  | 30                                   | 1.65              | 1.4 | 2.1  | 2.55               | 21.5 | 4.2 |
| Example 3                                  | 60                                       | 1.0 200° C., 24 hours | 30                                   | 2.2               | 1.9 | 1.6  | 2.0                | 2.0  | 2.5 |
| Example 4                                  | 60                                       | 10.0 do               | 30                                   | 3.0               | 1.3 | 1.65 | 1.5                | 1.45 | 3.0 |

S-HDET—Half-decay exposure time of the sample which shows the potential acceptance of 500 volts.

FIGURE 1 shows the changes of surface potential in a dark place of the photosensitive members of the examples in the invention and of the others for comparison. On the ordinate is plotted the surface potential in the logarithmic scale and, on the abscissa, the period of time passed after charging. Sample No. 4434 is a representative of Example 2. Sample No. 4470 represents Example 4. Sample No. 2384 is a representative of the photosensitive member of the powder which is not incorporated with cadmium iodide. All preparation conditions of Sample No. 2384 are the same as those of the sample incorporated with cadmium iodide, except for incorporation of iodide. In FIGURE 1, the curves noted with the mark O show the surface potential changes in the dark measured at the rest state (after placed in the dark place for more than 24 hours), the curves noted with the mark O show those measured at 300 seconds, after pre-exposure to 2000 lux for 2 minutes, and the curves with the mark Δ show those measured at 15 seconds, after pre-exposure to 2000 lux for 2 minutes. From this figure it becomes clarified that Sample No. 2384 for comparison can hardly be charged to be measured in the condition noted with the mark Δ, shows little potential acceptance only in the condition noted with the mark O, while the samples in the examples show re-

resulting in good copies with high image contrast and low background density.

#### Examples 7-20

Various kinds of metal iodides were added to the photoconductive powder comprising cadmium sulfide and carbonate CdS·1.5CdCO<sub>3</sub>, as alcohol solutions or aqueous solutions, in the same way as in the Examples 1-4 to prepare the photoconductive powder incorporated with metal iodide in accordance with the prescription described in Table 2. Then the photosensitive paints were prepared by dispersing the powder thus obtained in a binder material with porcelain ball mills in accordance with the prescription described in the Table 2. The binder material used herein was a kind of thermosetting acrylic resinous binder named "Magicron No. 200 Clear" manufactured by Kansai Paint Co., Ltd. In the same way as those described in Examples 1-4, the preparation of the photosensitive member for electrophotography, and the measurements of their characteristics were carried out.

The results are listed up in Table 2. Some samples in the examples showed the decreasing half-decay exposure time with the increasing thickness, though the potential acceptance increased with the increasing thickness of the photosensitive layer.

TABLE 2

| Metal Halides Added              | Ratio of<br>Binder to<br>Powder <sup>3</sup> | (-7.0 kv.) (sec.) |      |      | (+)7.0 kv.) (sec.) |      |      |
|----------------------------------|----------------------------------------------|-------------------|------|------|--------------------|------|------|
|                                  |                                              | A <sup>4</sup>    | B    | C    | A                  | B    | C    |
| Example 7 ZnI <sub>2</sub>       | 4.79                                         | 1/2               | 2.10 | 1.8  | 1.45               | 2.6  | 2.6  |
| Example 8 ZnI <sub>2</sub>       | 4.79 200° C., 24 hours                       | 1/2               | 0.50 | 0.43 | 0.50               | 1.5  | 1.5  |
| Example 9 AlI <sub>3</sub>       | 6.13                                         | 1/2               | 2.8  | 2.0  | 1.65               | 3.2  | 2.2  |
| Example 10 AlI <sub>3</sub>      | 6.13 200° C., 24 hours                       | 1/2               | 0.40 | 0.52 | -----              | 1.3  | 3.4  |
| Example 11 BiI <sub>3</sub>      | 8.85                                         | 1/2               | 2.9  | 2.9  | 2.5                | 3.0  | 2.3  |
| Example 12 BiI <sub>3</sub>      | 8.85 200° C., 24 hours                       | 1/2               | 0.65 | 0.50 | -----              | 1.8  | 1.6  |
| Example 13 SbI <sub>3</sub>      | 7.55                                         | 1/2               | 2.35 | 2.05 | 1.5                | 3.0  | 3.0  |
| Example 14 SbI <sub>3</sub>      | 7.55 200° C., 24 hours                       | 1/2               | 0.65 | 0.60 | -----              | 2.8  | 3.8  |
| Example 15 KI                    | 2.49                                         | 1/2               | 2.05 | 2.0  | 1.5                | 2.8  | 3.2  |
| Example 16 KI                    | 2.49 200° C., 24 hours                       | 1/2               | 0.92 | 0.5  | 0.6                | 1.7  | 1.75 |
| Example 17 HgI <sub>2</sub>      | 6.81                                         | 1/2               | 3.05 | 2.8  | 2.3                | 4.1  | 3.6  |
| Example 18 HgI <sub>2</sub>      | 6.81 200° C., 24 hours                       | 1/2               | 0.73 | 0.55 | 0.55               | 1.5  | 1.35 |
| Example 19 LiI·nH <sub>2</sub> O | 7.5                                          | 1/2               | 1.8  | 1.3  | 0.89               | 2.0  | 2.0  |
| Example 20 LiI·nH <sub>2</sub> O | 7.5 200° C., 24 hours                        | 1/2               | 0.8  | 0.75 | 0.58               | 1.55 | 1.2  |

<sup>1</sup> Half-decay exposure time of the electrophotographic photosensitive member which shows the potential acceptance of 500 volts.

<sup>2</sup> Metal halide was added to 242 grams of the powder.

<sup>3</sup> Binder material was mixed with the powder incorporated with metal halide at the weight ratio described.

<sup>4</sup> The baking conditions of the coatings A: 150° C., 30 min.; B: 200° C., 60 min.; C: 250° C., 30 min.

markable improvement, though they have a little light 60 fatigue effect still.

#### Examples 5 and 6

Two photosensitive drums were prepared by coating aluminum tubes with the photosensitive paint of Example 4, drying the coating at 70° C. for 50 minutes and baking them at 150° C. for 30 minutes. The coating thicknesses of the photosensitive layers of the drums were about 3.2 mg./cm.<sup>2</sup> for Sample No. A-111 in Example 5 and about 6.13 mg./cm.<sup>2</sup> for Sample No. A-113 in Example 6 after baking. The surface potentials before and after exposing were measured and their changes during repeated use were examined by charging with -6.5 kv. corona discharge and exposing them to about 100 lux. sec. as they were rotated at a revolution rate of 6 r.p.m. The results are shown in the FIGURE 2. In 75

#### EXAMPLE 21

In 100 grams of a binder material of a kind of thermosetting acrylic resin called "Magicron No. 200 Clear" (solid part being about 50%) and 120 mls. of thinner, 3.1 grams of aluminum iodide, AlI<sub>3</sub>, was dissolved. Then, in this binder containing AlI<sub>3</sub>, there was dispersed 100 grams of powder comprising CdS·CdCO<sub>3</sub> to provide a photosensitive paint, which was coated on aluminum sheets, dried at 70° C. and then baked at 200° C. for 30 minutes to form photosensitive members.

The electrophotographic characteristics of the photosensitive members thus obtained were evaluated in the same manner as described in the Examples 1-4, resulting in photosensitivity about 2.5 times as high as those of the photosensitive member not containing aluminum iodide.

What is claimed is:

1. A photoconductive insulating material consisting essentially of photoconductive powder particles and an electrically insulating binder selected from the group consisting of organic resinous binders and low melting point glasses in which the said photoconductive powder particles are dispersed, said powder particles consisting mainly of cadmium sulfide-cadmium carbonate photoconductive material (that is,  $\text{CdS} \cdot n\text{CdCO}_3$ ,  $n < 4$ ) having a metal iodide incorporated therewith, said metal iodide being selected from the group consisting of water soluble iodides, organic solvent soluble iodides, and iodides which form a vapor upon heating and where the molar ratio of said metal iodide to said cadmium sulfide-cadmium carbonate photoconductive material extends from approximately 0.01 to 0.1.

2. A material in claim 1 where  $n$  is 1.5 and the said molar ratio is 0.1.

3. A material as in claim 1 where the metal of said metal iodide is selected from the group consisting of cadmium, zinc, aluminum, bismuth, tin, potassium, mercury, and lithium.

References Cited

UNITED STATES PATENTS

|           |         |                |          |
|-----------|---------|----------------|----------|
| 2,866,878 | 12/1958 | Briggs et al.  | 2.52—501 |
| 3,324,299 | 6/1967  | Schuil         | 252—501  |
| 3,345,161 | 10/1967 | Mammino et al. | 96—1.5   |

MAYER WEINBLATT, Primary Examiner

W. E. SCHULZ, Assistant Examiner

U.S. Cl. X.R.

96—1.5